

## UNITED STATES PATENT OFFICE

2,482,382

## CORROSION RESISTANT ALLOY

Ralph W. Thomas, Waukesha, Wis., assignor to  
 Waukesha Foundry Company, Waukesha, Wis.,  
 a corporation of Wisconsin

No Drawing. Application June 12, 1947,  
 Serial No. 754,280

2 Claims. (Cl. 75—170)

1

This invention relates to a corrosion resistant alloy.

It is a primary object of the invention to provide an alloy which is particularly suited for use in dairy equipment and other food industries in that it contains neither copper nor iron, has high tensile strength and substantial Brinell hardness, is readily cast and easily machined, and has good bearing qualities in that it moves freely upon itself or upon stainless steel without galling.

For machinery used in the handling of dairy products and other foods where sanitation is important, it is common to use alloys which do not corrode. Those most commonly employed are nickel alloys and stainless steel. The nickel alloys commonly have a copper base and there is some prejudice against the use of an alloy containing copper in the handling of foods. Stainless steel, however, has the unfortunate quality of galling. That is to say, one piece cannot rub upon another without becoming roughened and seizing.

The preferred analysis of my improved alloy is as follows:

|           | Per cent |
|-----------|----------|
| Nickel    | 78.00    |
| Lead      | 4.00     |
| Zinc      | 8.00     |
| Tin       | 8.00     |
| Manganese | 2.00     |

Some variation in the composition is permissible but for most satisfactory results the percentages of the ingredients should be held within the following limits:

|           | Per cent |
|-----------|----------|
| Nickel    | 76-79    |
| Lead      | 3-5      |
| Zinc      | 7-9      |
| Tin       | 6.5-8.5  |
| Manganese | 1.5-2.0  |

An alloy made in accordance with the present

invention not only contains no copper or iron, but is highly resistant to corrosion, has adequate strength, casts and machines readily and does not seize or gall when run in contact with itself or other alloys including stainless steel.

When the ingredients are mixed in approximately the stated proportions, the following data will describe its additional physical properties:

|                  |                             |
|------------------|-----------------------------|
| Tensile strength | 50,000-60,000 p. s. i.      |
| Yield point      | 40,000-45,000 p. s. i.      |
| Elongation       | (per cent in 2 inches) 7-10 |
| Brinell hardness | (3000 kg.)—150              |

Where it is not required that the alloy be cast, the manganese may be omitted and an equal additional amount of nickel substituted. The essential ingredients are nickel, lead, zinc and tin, the nickel representing more than three-fourths of the total.

I claim:

1. A copper and iron-free corrosion resistant and castable alloy for use in food processing machinery and consisting of 76 to 79% nickel, 7 to 9% zinc, 6.5 to 8.5% tin, 3 to 5% lead and 1.5 to 2% manganese.

2. A copper and iron-free corrosion resistant and castable alloy for use in food processing machinery and consisting of 78% nickel, 8% zinc, 8% tin, 4% lead and 2% manganese.

RALPH W. THOMAS.

## REFERENCES CITED

The following references are of record in the file of this patent:

| UNITED STATES PATENTS |               |               |
|-----------------------|---------------|---------------|
| Number                | Name          | Date          |
| 1,924,244             | Koster        | Aug. 29, 1933 |
| 1,988,154             | Bolton et al. | Jan. 15, 1935 |
| 2,239,144             | Dean et al.   | Apr. 22, 1941 |